

Jan. 26, 1954

J. W. DONEGAN

2,667,460

MANUFACTURE OF ACTIVATED CARBON

Filed Feb. 28, 1951



INVENTOR.  
JOSEPH W. DONEGAN

BY  
*Alvin Engelstein*  
ATTORNEY.

## UNITED STATES PATENT OFFICE

2,667,460

## MANUFACTURE OF ACTIVATED CARBON

Joseph W. Donegan, New Brunswick, N. J., assignor to Allied Chemical & Dye Corporation, New York, N. Y., a corporation of New York

Application February 28, 1951, Serial No. 213,164

8 Claims. (Cl. 252—421)

## 1

This invention relates to the manufacture of activated carbons from tars and pitches and more particularly refers to a new and improved method of converting the tars and pitches into high yields of activatable char.

In the distillation of crude tars to produce desirable carbolic and creosote oil distillates, a problem of disposing of the resultant pitch residues often exists. The utilization of such residues as fuels represents a substantial depreciation in value of the bituminous products with consequent effective increase in cost for production of the distillates. As described in my co-pending application Serial No. 18,712, filed April 2, 1948, now Patent 2,549,298, issued April 17, 1951, I have developed a method of separating solid carbonaceous materials susceptible to activation from tars and pitches by the addition of solvent thereto and by subsequent processing to convert the solid carbonaceous materials into activated carbon which has a greatly enhanced value compared to the tar or pitch from which it was derived. The yield of solid carbonaceous materials removed from the tars and pitches for activation ranges from about 10 to 40% by weight dependent upon the nature of the particular tar or pitch employed.

An object of the present invention is to provide a method for converting coal tar pitches, water-gas tar pitches and oil-gas tar pitches into high yields of activated carbon with a reduced amount of by-products.

Another object of the invention is to produce increased yields of solid carbonaceous materials from coal tar pitches, water-gas tar pitches and oil-gas tar pitches without the use of solvents.

Other objects and advantages of the present invention will be apparent from the following description and accompanying drawing.

In general, the present invention involves blowing air through a molten body, i. e. liquid phase, of residual hydrocarbon material boiling above 670° F. until the benzol-insoluble content of the hydrocarbon material is increased to at least 55% by weight, pulverizing the air-blown hydrocarbon material to at least 80% passing a No. 200 sieve, and calcining the pulverized hydrocarbon material until an infusible activatable char is obtained and then activating the char by steam or flue gases. The pulverulent activated char thus obtained is particularly suitable for decolorizing purposes. If it is desired to produce granular activated char suitable as a vapor adsorbent, the pulverized air-blown hydrocarbon material is compressed to form bri-

## 2

quettes which are then crushed and sized to the desired size granules and the latter calcined and activated to activated char.

More specifically, increased yields of activatable char may be obtained from coal tar, water-gas tar and oil-gas tar by separating from the tars a high boiling hydrocarbon material substantially free from oils boiling below 670° F. and having a melting point (cube method) with-  
 5 in the range of 150° F. to 325° F., preferably between 160° to 250° F., heating the high boiling hydrocarbon to maintain it in a molten condition, passing air or other oxygen-containing gas in contact with said molten hydrocarbon material maintained in an agitated state at a temperature between 550° and 950° F., preferably 650° to 850° F. for a sufficient length of time to increase the benzol-insoluble content of the hydrocarbon material to in excess of 55%, desir-  
 10 ably below 90% and preferably between 65 to 85%, pulverizing the air-blown hydrocarbon material to preferably below 200 mesh, compressing the pulverized hydrocarbons at pressures preferably ranging from 5000 to 50,000 p. s. i. to  
 15 form briquettes, crushing and sizing the briquettes into granules of, e. g., 10 to 20 mesh size, calcining the granules in the presence of oxygen-  
 20 containing gas at temperatures sufficiently high to char the granules, preferably at increasing temperatures from below about 400° F. to within the range of 400°-850° F., desirably avoiding temperatures in excess of 750° F., while maintaining the temperature sufficiently low during such calcination so that the granules  
 25 remain in an unfused condition, continuing the calcination until an infusible activatable char is obtained, and activating the char at an elevated temperature, generally from 1450° to 2200° F., by the action of steam or flue gases.  
 30  
 35  
 40 Tars are conventionally subjected to fractional distillation to separate them into cuts of different boiling points. A typical coke-oven tar will yield on distillation the following:

|                 | Per cent (by volume) |
|-----------------|----------------------|
| 45 Carbolic oil | 16                   |
| Creosote oil    | 25                   |
| Heavy oil       | 15                   |
| Fuel pitch      | 41                   |
| Loss            | 3                    |

The carbolic oil and creosote oil are in demand and bring a high market price. The heavy oil is unsalable as creosote, and is frequently disposed of as fuel, with accompanying loss of value. Likewise, fuel pitch, for the most part has the

relatively low value of fuel. I have found that in the practice of my process the undesirable heavy oil can be converted into superior grades of activated carbon and further a greater yield of activated carbon from fuel pitch can be produced than hitherto had been obtained.

The charging stock subjected to treatment in my process may be coal-tar pitch or water-gas tar pitch or oil-gas tar pitch or mixtures of these pitches; such pitches containing substantially no oils boiling below 670° F. and having a melting point (cube method) between 150° F. and 325° F., preferably 160° to 250° F. The charging stock may be obtained conveniently by distillation, for example, of a typical coke-oven tar into the following cuts:

|              | Per cent (by volume) |
|--------------|----------------------|
| Carbolic oil | 16                   |
| Creosote oil | 25                   |
| Pitch        | 56                   |
| Loss         | 3                    |

In this distillation only two distillate fractions are obtained, the heavy oil and fuel pitch fractions of the preceding example together comprising the residual pitch. This residual pitch is eminently suitable for conversion into activated carbon.

The accompanying drawing is a diagrammatic flow diagram illustrating the process of the present invention.

Referring to the drawing, the charging stock which may be a coal-tar pitch, water-gas pitch or oil-gas pitch derived from the corresponding tars is introduced from storage container 1 through opening 2 into the top of blow still 3. Due to expansion of the charge upon heating and blowing of air therethrough, it is advisable not to fill blow still 3 to a level higher than about  $\frac{2}{3}$  of its height. As illustrated in the drawing, the blow still, generally designated by numeral 3, consists of a vertical cylindrical chamber 4 equipped with a power driven agitator 5 of the paddle type. Air or other oxygen-containing gas may be introduced into the top of vertical hollow shaft 6 of agitator 5 and discharged into the body of pitch in blow still 4 through a perforated cross pipe 7 at the terminal end of shaft 6 near the bottom chamber 4. Gases and vapors are released from the top of still 3 through opening 8. Heat may be applied to the contents of vessel 4 by generating combustion gas in a conventional furnace 9 and passing the hot combustion gas through the annular space bounded by the walls of chamber 4 and jacket 11 and thence discharging the spent combustion gas through stack 12.

In operation the pitch in blow still 3 is heated to a molten condition, i. e. a liquid phase state, by the transfer of heat from hot combustion gases passing around chamber 4. Air is blown into hollow shaft 6, out through perforated pipe 7, and thence up through the body of molten pitch in still 4. Rotation of agitator 5 insures intimate contact between the molten pitch and air rising therethrough, and further maintains more uniform temperature conditions throughout the body of molten pitch. During the reaction the temperature of the still contents is maintained between 550° and 950° F. and may be regulated in a manner well known in the art by controlling the amount and temperature of hot combustion gases passing around still 4. Although temperatures below 550° F. may be employed, the reaction at this lower temperature is unduly long. At temperatures above 950° F. distillation losses are

increased and, in addition, operation at these higher temperatures presents a fire hazard. A preferred temperature range of 650° to 850° F. was found convenient and satisfactory in practical operation. The rate of air introduction into the molten hydrocarbon material in blow still 4 influences the time required to consummate the reaction. At a low rate the reaction time would be impractically long, and at too high a rate of air introduction it would be difficult to control the temperature of the molten pitch. In commercial practice air introduced in contact with the molten pitch at the rate of 20 to 50 cubic feet per minute per ton of pitch will in general be found to give good results.

Air is continuously blown down through hollow shaft 6 and out through the perforations in pipe 7 into the molten pitch maintained at a temperature between 550° and 950° F. until the benzol-insoluble content of the pitch in blow still 4 exceeds 55%. The benzol-insoluble content of the molten pitch in still 4 may readily be determined by analyzing small samples withdrawn from the body of pitch. As a practical matter, once an operator has acquired experience with a particular pitch and the temperature, time and air rate conditions necessary to convert the pitch to a material having a benzol-insoluble content in excess of 55%, it becomes unnecessary for him to analyze samples during the operation and he need only duplicate the conditions to which similar pitch had previously been subjected. Ordinarily, it will be found that the benzol-insoluble content of the pitch increases to approximately 65% at the end of five hours, 75% at the end of 6 hours and 85% at the end of 7½ hours. It is inadvisable to continue the air blowing to produce a product having a benzol-insoluble content in excess of 90% because the pitch becomes plastic and dough-like and most difficult to maintain in an agitated condition. At the start of the operation the molten pitch is in a rather fluid state, and during the course of the reaction the pitch becomes increasingly viscous and of higher melting point, in the nature of a fused mass. On cooling the fused mass is generally dense and vitreous and usually brittle and coke-like in appearance. The yield of air blown pitch resulting from the reaction in blow still 4 is quite high, usually in excess of 70% and more generally 80-85% by weight of the charge of pitch undergoing treatment in still 4 from which it will be apparent that a relatively small proportion of undesirable by-products is produced.

As a result of passing air through the body of molten pitch in still 4 and heating of the pitch there is evolved from the body of pitch residual gases such as nitrogen, unreacted oxygen, carbon monoxide, carbon dioxide together with low boiling hydrocarbon vapors carried by the residual gases. The gases and vapors are released from the top of blow still 4 through opening 8 and directed through conduit 13 into a conventional condenser not shown in the drawing wherein the gases are cooled by indirect heat exchange with a cooling medium such as water and the vapors are condensed to form a liquid condensate which is collected and may be burned as fuel or disposed of otherwise.

After completion of the reaction, the air-blown pitch is cooled and solidified by discharging the still contents while in a heated fluid condition from the bottom of blow still 4 through line 14 into pitch-bay 10 which latter is simply a shallow open tank. Cooling and solidification of the

pitch may also be accomplished by the use of a conventional flaking drum not shown in the drawing.

The solidified pitch is directed through conveyor 28 to a suitable pulverizer 15 wherein the pitch is ground so that substantially all the finely pulverized pitch passes a 200 sieve. A gaseous propelling means is frequently used in many of the commercial pulverizing devices, designated by numeral 15, with the result that separation of the gaseous propellant from finely divided solids must be effected. This may be accomplished by passing the gaseous propellant carrying the pulverized pitch through conduit 16 into dust collector 17 which may be of the conventional cyclone type. The gaseous propellant is released from the top of dust collector 17 through opening 18 and the pulverized pitch permitted to settle in the bottom of collector 17.

The pitch dust from dust collector 17 is 20 briquetted in conventional compressing machines designated as briquette press 21 at pressures ranging from 5,000 to 50,000 p. s. i. depending upon the physical structure and density desired in the ultimate product. The briquettes are then ground in a conventional granulator 22 to about 4 to 25 mesh grain after which the ground briquettes are sized in the usual manner in screen 23. The sized material from screen 23 is then conveyed to calciner 24, desirably a rotary externally heated retort, wherein charring is effected by passing the stream of air or other oxygen-containing gas through the retort in contact with the granular material at gradually increasing temperature from below 400° F., preferably from 300° F. to within the range of 400°-750° F. Calcination of the granular material is carried out under the conditions of heating just described until there is obtained an infusible char without permitting fusion of the granules or leaving incompletely reacted and fusible residues. Ordinarily effective calcination of the granular material will be accomplished in 2 to 8 hours.

The charred material may be finally activated by subjecting it in activator 25 to the action of steam or flue gases by known procedures while maintaining temperatures of the general order of 1450°-2200° F.

From the foregoing the advantages of the present process will be apparent in that heavy oil previously suitable only as a low value fuel product is converted into valuable activated carbon, fuel pitch is converted into higher yields of activated carbon, production of undesirable by-products is minimized, and the use of solvents for extracting the benzol-soluble material from pitches is eliminated.

In order to clearly show the differentiation between air blowing of pitch in accordance with the present invention and normal pyrolysis of pitch as is conventional in the art, a coke obtained by simple pyrolysis of coal tar pitch in a retort, in the absence of air, was compared with the product of air blowing as a raw material for activated carbon production. Both materials were pulverized, briquetted, granulated, screened and calcined according to the same procedure except that in the briquetting step the pyrolytic coke required addition of about 10% tar as a binder, and even then the pellets were very weak, whereas the briquetting of the air-blown pitch was effected without binder and gave strong, hard pellets. Following calcination, the air-blown pitch and pyrolytic coke pellets were steam-activated at 1790° F. and these products 75

were then evaluated by the standard iodine absorption procedure. The activated pyrolytic coke and air-blown pitch had iodine values of 29.6 and 79.9, respectively. The high activity from the product of air-blown pitch clearly differentiates the air-blown pitch from the coke as a starting material for activated carbon manufacture.

The following examples illustrate the present invention.

#### Example 1

A coke-oven tar obtained from the pyrolytic decomposition of bituminous coal was subjected to distillation until all the hydrocarbon material boiling below 680° F. was evolved as vapors, constituting 55% by volume of the coke oven tar, leaving as residue a soft plastic pitch having a melting point of 180° F. The 180° F. pitch was placed in an externally heated vertical vessel and heat applied to the walls of the vessel until the pitch became molten and its temperature raised to 710° F. Air was blown through the constantly agitated body of molten pitch maintained at 700°-710° F. at a rate of 32 cubic feet per minute per ton of pitch for seven hours at the end of which time a yield of 85% blown pitch analyzing 82% benzol-insoluble was obtained. The air-blown pitch was then pulverized to pass a 200 mesh sieve, the powdered pitch briquetted at 5,000 p. s. i., and the briquettes granulated to 10-20 mesh grain. The granulated briquettes were charged to a rotary retort and air passed therethrough while the temperature was gradually increased (over about 5 hours) from 400° F. to 750° F. The resultant char was unfused and infusible, wholly insoluble in benzol. Activation of this granular char at 2010° F. with steam gives an activated carbon whose activity is such that 0.5 gram removed 85% of the color from 100 ml. of a standard brown sugar solution.

#### Example 2

A pitch of 200° F. melting point, obtained by distillation of a crude heavy water-gas tar, was blown with air at 752° F. and an air rate of 35 cu. ft./ton/min. for 6 hours. A yield of 78% of a pitch analyzing 72.8% benzol-insoluble was obtained. This pitch was pulverized to pass the 200 sieve, briquetted at 5,000 p. s. i. and the briquettes granulated and screened to obtain a 10-20 mesh fraction. The granulated, briquetted pitch was charged to a rotary retort and gradually heated, over a period of about 5 hours, from 400 to 750° F. The resultant char was infusible, and activated readily when reacted with steam at 1800° F. The activity of the product was such that 0.25 gram removed 77% of the iodine from a standard test solution containing 270 mg. of iodine per hundred ml.

#### Example 3

A pitch obtained by distillation of an oil-gas tar had a melting point of 256° F. and a benzol-insoluble content of 41%. After air blowing at 752° F. for 6 1/4 hours, a pitch analyzing 84% benzol-insoluble was obtained. This latter pitch product was pulverized to pass the 200 mesh sieve, briquetted at 5,000 p. s. i. and granulated to obtain a 10-20 mesh fraction. The granular product was calcined in air as in the previous examples and was then activated with steam at 1790° F. The activated product had an iodine value of 87%.

#### Example 4

A coke-oven tar pitch having a benzol-insolu-

ble content of 31.9% was blown with air at a rate of 32 cubic feet per ton per minute for 3½ hours to a benzol-insoluble content of 80%. It was pulverized to such fineness that 80% passed a No. 200 sieve, briquetted at 5,000 p. s. i., and granulated to 10-25 mesh. The granulated briquettes were calcined in air at gradually increasing temperatures of 400°-750° F. in about 5 hours. The resultant char was activated with steam at 1800° F. and had an iodine value of 81.5% and adsorbed 53% of its own weight of carbon tetrachloride when in equilibrium with an air stream containing 40,000 p. p. m. of that vapor at 77° F.

Although certain preferred embodiments of the invention have been disclosed for purpose of illustration it will be evident that various changes and modifications may be made therein without departing from the scope and spirit of the invention.

I claim:

1. A process for the production of activatable char from high boiling hydrocarbon material derived from pyrolytic decomposition products selected from the group consisting of coal tar, water-gas tar and oil-gas tar which comprises subjecting said pyrolytic decomposition products to distillation to remove therefrom substantially all the oils boiling below 670° F., passing air in intimate contact with the residual hydrocarbon material maintained at a temperature between 650 and 850° F. at a rate of 20 to 50 cubic feet per minute per ton of residual hydrocarbon material for a sufficient length of time to convert said residual hydrocarbon material into a product having a benzol-insoluble content of 65 to 85% by weight, pulverizing the air-blown hydrocarbon material to below about 200 mesh size, compressing the pulverized hydrocarbons at pressures ranging from 5000 to 50,000 p. s. i. to form briquettes, crushing and sizing the briquettes into granules of about 4 to 20 mesh size, calcining the granules in the presence of oxygen-containing gas at increasing temperatures from below about 400° F. to not in excess of 850° F. while maintaining the temperatures sufficiently low during such calcination so that the granules remain in an unfused condition, continuing the calcination until an infusible activatable char is obtained, and activating the char at a temperature from 1450° to 2200° F.

2. A process for the production of activatable char from coal tar which comprises subjecting said coal tar to distillation to remove therefrom substantially all the oils boiling below 670° F., passing air in intimate contact with the residual coal tar pitch maintained at a temperature between 650° and 850° F. at a rate of 20-50 cubic feet per minute per ton of residual coal tar pitch for a sufficient length of time to convert said coal tar pitch into a product having a benzol-insoluble content of 65-85% by weight, pulverizing the air-blown pitch to below about 200 mesh, compressing the pulverized pitch at pressures ranging from 5000 to 50,000 p. s. i. to form briquettes, crushing and sizing the briquettes into granules of about 4 to 20 mesh size, calcining the granules in the presence of oxygen-containing gas at increasing temperatures from below about 400° F. to not in excess of 850° F. while maintaining the temperatures sufficiently low during such calcination so that the granules remain in an unfused condition, containing the calcination until an infusible activatable char is obtained and

activating the char at a temperature from 1450° to 2200° F.

3. A process for the production of activatable char from water-gas tar which comprises subjecting said water-gas tar to distillation to remove therefrom substantially all the oils boiling below 670° F., passing air in intimate contact with the residual water-gas tar pitch maintained at a temperature between 650° and 850° F. at a

10 rate of 20-50 cubic feet per minute per ton of residual water-gas tar pitch for a sufficient length of time to convert said water-gas tar pitch into a product having a benzol-insoluble content of 65-85% by weight, pulverizing the air-blown

15 pitch to below about 200 mesh, compressing the pulverized pitch at pressures ranging from 5000 to 50,000 p. s. i. to form briquettes, crushing and sizing the briquettes into granules of about 4 to 20 mesh size, calcining the granules in the presence of oxygen-containing gas at increasing temperatures from below about 400° F. to not in excess of 850° F. while maintaining the temperatures sufficiently low during such calcination so that the granules remain in an unfused condition, continuing the calcination until an infusible activatable char is obtained and activating the char at a temperature from 1450° to 2200° F.

4. A process for the production of activatable char from oil-gas tar which comprises subjecting said oil-gas tar to distillation to remove

30 therefrom substantially all the oils boiling below 670° F., passing air in intimate contact with the residual oil-gas tar pitch maintained at a temperature between 650° and 850° F. at a rate of 20-50 cubic feet per minute per ton of residual oil-gas tar pitch for a sufficient length of time to convert said oil-gas tar pitch into a product having a benzol-insoluble content of 65-85% by weight, pulverizing the air-blown pitch to below

35 about 200 mesh, compressing the pulverized pitch at pressures ranging from 5000 to 50,000 p. s. i. to form briquettes, crushing and sizing the briquettes into granules of about 4 to 20 mesh size, calcining the granules in the presence of oxygen-containing gas at increasing temperatures from

40 below about 400° F. to not in excess of 850° F. while maintaining the temperatures sufficiently low during such calcination so that the granules remain in an unfused condition, continuing the calcination until an infusible activatable char is obtained and activating the char at a temperature from 1450° to 2200° F.

45 5. A process for the production of activatable char from high boiling hydrocarbon material derived from pyrolytic decomposition products selected from the group consisting of coal tar, water-gas tar and oil-gas tar which comprises subjecting said pyrolytic decomposition products to distillation to remove therefrom substantially

50 all the oils boiling below 670° F., passing air in intimate contact with the residual hydrocarbon material maintained at a temperature between 650 and 850° F. at a rate of 20 to 50 cubic feet per minute per ton of residual hydrocarbon material for a sufficient length of time to convert

55 said residual hydrocarbon material into a product having a benzol-insoluble content of 65 to 85% by weight, pulverizing the air-blown hydrocarbon material to below about 200 mesh size,

60 calcining the pulverized hydrocarbon material in the presence of oxygen-containing gas at increasing temperatures from below about 400° F. to not in excess of 850° F. while maintaining the temperatures sufficiently low during such calcination so that the hydrocarbon material remains in

65

70

75

an unfused condition, continuing the calcination until an infusible activatable char is obtained, and activating the char at a temperature from 1450° to 2200° F.

6. A process for the production of activatable char from coal tar which comprises subjecting said coal tar to distillation to remove therefrom substantially all the oils boiling below 670° F., passing air in intimate contact with the residual coal tar pitch maintained at a temperature between 650° and 850° F. at a rate of 20-50 cubic feet per minute per ton of residual coal tar pitch for a sufficient length of time to convert said coal tar pitch into a product having a benzol-insoluble content of 65-85% by weight, pulverizing the air-blown pitch to below about 200 mesh, calcining the pulverized hydrocarbon material in the presence of oxygen-containing gas at increasing temperatures from below about 400° F. to not in excess of 850° F. while maintaining the temperatures sufficiently low during such calcination so that the hydrocarbon material remains in an unfused condition, continuing the calcination until an infusible activatable char is obtained and activating the char at a temperature from 1450° to 2200° F.

7. A process for the production of activatable char from water-gas tar which comprises subjecting said water-gas tar to distillation to remove therefrom substantially all the oils boiling below 670° F., passing air in intimate contact with the residual water-gas tar pitch maintained at a temperature between 650° and 850° F. at a rate of 20-50 cubic feet per minute per ton of residual water-gas tar pitch for a sufficient length of time to convert said water-gas tar pitch into a product having a benzol-insoluble content of 65-85% by weight, pulverizing the air-blown pitch to below about 200 mesh, calcining the pulverized hydrocarbon material in the

presence of oxygen-containing gas at increasing temperatures from below about 400° F. to not in excess of 850° F. while maintaining the temperatures sufficiently low during such calcination so that the hydrocarbon material remains in an unfused condition, continuing the calcination until an infusible activatable char is obtained and activating the char at a temperature from 1450° to 2200° F.

- 10 8. A process for the production of activatable char from oil-gas tar which comprises subjecting said oil-gas tar to distillation to remove therefrom substantially all the oils boiling below 670° F., passing air in intimate contact with the residual oil-gas tar pitch maintained at a temperature between 650° and 850° F. at a rate of 20-50 cubic feet per minute per ton of residual oil-gas tar pitch for a sufficient length of time to convert said oil-gas tar pitch into a product having a benzol-insoluble content of 65-85% by weight, pulverizing the air-blown pitch to below about 200 mesh, calcining the pulverized hydrocarbon material in the presence of oxygen-containing gas at increasing temperatures from below about 400° F. to not in excess of 850° F. while maintaining the temperatures sufficiently low during such calcination so that the hydrocarbon material remains in an unfused condition, continuing the calcination until an infusible activatable char is obtained and activating the char at a temperature from 1450° to 2200° F.
- 15 20 25 30 35 40

JOSEPH W. DONEGAN.

References Cited in the file of this patent

UNITED STATES PATENTS

| Number    | Name    | Date          |
|-----------|---------|---------------|
| 2,008,146 | Morrell | July 16, 1935 |
| 2,549,298 | Donegan | Apr. 17, 1951 |